

2,888,399

PROCESS FOR INHIBITING CORROSION IN OIL  
AND GAS WELLS

Arthur F. Wirtel, Glendale, and Charles M. Blair, Jr., Webster Groves, Mo., assignors to Petrolite Corporation, Wilmington, Del., a corporation of Delaware

No Drawing. Application April 1, 1953  
Serial No. 346,264

1 Claim. (Cl. 252—8.55)

This invention relates to the inhibition of corrosion of metals. It includes new compositions for use in preventing corrosion of metals, in particular, iron, steel, and ferrous alloys, and the process of preventing such corrosion by application of the new compositions to the surfaces of the metals. The invention is of particular value in the prevention of corrosion of pipe or equipment which is in contact with corrosive oil-containing media as, for example, in oil wells producing corrosive oil or oil-brine mixtures, in oil refineries, and the like, but it is useful in numerous other systems or applications, as the new compositions appear to possess properties which impart to metals resistance to attack by a variety of corrosive agents, such as brines, weak inorganic acids, or organic acids,  $\text{CO}_2$ ,  $\text{H}_2\text{S}$ , etc.

A wide range of corrosion inhibitors, particularly for use in oil and gas wells, oil refineries and the like, have heretofore been used or suggested for use. One group is that which includes amines, amido-amines and nitrogen heterocyclics characterized by the presence of two or more nitrogen atoms, at least one of which is basic, and one or more hydrocarbon groups having from 8 to 32 carbon atoms. Such compounds have a moderately strong nitrogen-containing basic group (either free or in salt form), which may be present as part of a heterocyclic ring structure, as in certain amidine, e.g., imidazoline, tetrahydropyrimidine and carbamyl compounds, or not, as in non-cyclic amino amides or polyamines. There is a substantial variation in the relative effectiveness of such agents as corrosion inhibitors. In general, we have found that the more complex products having a plurality of basic nitrogen atoms, and in particular relatively complex amino-amides, imidazolines, tetrahydropyrimidines and carbamyl derivatives of cyclic amidines are more effective than simpler amino compounds.

The present invention is based upon the discovery that the anticorrosive action of such agents, as a class, is markedly enhanced if they are associated with an alkylated aromatic sulfonic acid of the type hereinafter defined, or a salt thereof. We have no explanation of this observed result, as in our tests, we have not found that the alkylated aromatic sulfonic acids which we use, or their salts, have any marked corrosion inhibiting action. On the other hand, we have found corrosion inhibitors, which when used conventionally reduce corrosion very substantially, have their corrosion inhibiting action markedly enhanced by admixture with about 50% of an alkylated aromatic sulfonic acid salt. Thus, in one instance, we found that a known corrosion inhibitor (a mixture of mono- and diimidazolines obtained by heating 384 pounds of tall oil and 146 pounds of triethylene tetramine for 2½ hours at 285° C., which possibly contained a minor proportion of amides in addition to the imidazolines) when injected at the rate of 2½ gallons a week into a gas-distillate well reduced the iron content of water from the flow line at the surface from about 240 p.p.m. to 50–60 p.p.m. With this same inhibitor, injected at the same rate, but in admixture with about ½ its weight of

ammonium diisopropyl naphthalene sulfonate, the iron content of the water was reduced to about 10–15 p.p.m. In both cases, suitable solvents were used and the inhibiting composition was introduced down the annulus between the casing and the tubing. The ammonium diisopropyl naphthalene sulfonate had no substantial corrosion inhibiting properties.

Thus, the new compositions of the invention consist of admixtures of (1) a corrosion-inhibiting agent characterized by having at least two nitrogen atoms, at least one of which is basic, which may be amino groups or form portions of heterocyclic ring structures and at least one hydrocarbon group having 8 to 32 carbon atoms, with (2) an alkylated aromatic sulfonic acid, which may be represented by the formula



in which R is an alkyl radical having 3 to 12 carbon atoms, n is a number from 1 to 3, and with the requirement that the total number of carbon atoms present in  $(\text{R})_n$  is at least 6, or the formula



in which n is one or two, R is an alkyl group having 3 to 18 carbon atoms and with the requirement that the total number of carbon atoms in  $(\text{R})_n$  is at least 9. The nature of the cation does not seem to be of particular consequence. It can be hydrogen, sodium, potassium, ammonium, the cation of a water-soluble amine, such as monoethanol amine, diethanol amine, or triethanol amine, or the cation of a water-insoluble amine, such as amyl amine, cyclohexyl amine, benzyl amine, amines derived from higher fatty acids having 8 to 18 carbon atoms, such as lauryl amine or the mixed amines derived from fats or oils, which are commercially available, or other cation, including polyamines or the like, such as ethylenediamine, in which case the polybasic ion can be combined with one or more sulfonic acid groups up to a number equal to its number of basic groups, e.g., in the case of ethylene diamine, either one or two moles, or some intermediate amount, of sulfonic acid per mole of diamine. If the cation is hydrogen it is possible that this agent may form salts with the corrosion-inhibiting amine, but in most instances, we think that the corrosion inhibiting amine and the sulfonic acid or sulfonate will be present in simple admixture, as the corrosion inhibiting amine will generally, and advantageously, be used in the form of a salt, as will the sulfonic acid.

In addition to these two essential constituents of the new compositions, there will normally be present additional conventional materials, such as solvents where the admixtures are to be used in liquid form, waxes or other solidifying agents where the products are to be used in solid stick form, and waxes or other solidifying agents and a weighting material, such as barium sulfate or lead oxide, where the compositions are to be used in the form of weighted sticks. The use of corrosion inhibitors, particularly for oil and gas well treatment, in liquid form, or in stick form with or without weighting agents, is conventional and well known, and the present invention is concerned, not with the form of application of the compositions, but with the enhancement of the corrosion inhibiting action of the nitrogen-containing agent by association therewith of the specified alkylated aromatic sulfonic acid.

In general, we have found that minor proportions of

the alkylated aromatic sulfonic acid based on the corrosion inhibiting compound are adequate to produce marked enhancement of the activity of the composition. Thus, 10% or less of an alkylated aromatic sulfonic acid, based on the inhibitor, produces a marked effect. At present, we are not aware of any requirement as to an upper limit. It, so far as we are aware, will be fixed by economic considerations, as use of an excess of an alkylated aromatic sulfonic acid does not reduce the enhancement of the anticorrosion activity, nor do amounts in excess of 50 to 100%, based on the corrosion inhibitor, appear to increase the enhancement beyond that obtained with 10 to 50%. At worst, an excess serves as an additional diluent. Thus, the range we contemplate is from about 5% to about 100% of the alkylated aromatic sulfonic acid, based on the corrosion inhibitor, but it is to be understood that use of larger amounts does not involve departure from the invention.

As previously stated, the corrosion inhibitors used in the new compositions are characterized by the presence of (1) at least one hydrocarbon group having 8 to 32 carbon atoms, and (2) at least two nitrogen atoms, of which at least one is basic, which may be present as part of a heterocyclic ring structure or not. In certain of the most effective inhibiting agents, basic nitrogen atoms are present as part of the heterocyclic ring structure and also as part of a side chain substituted on the heterocyclic ring structure, as for example, in the imidazolines derived from polyalkylene polyamines having 3 or more basic amino groups, e.g., the high-boiling residue from the preparation of ethylene diamine and the like. A number of such compounds are known to serve as corrosion inhibitors. We have found that, as a class, their corrosion inhibiting efficiency is enhanced by associating them with an alkylated aromatic sulfonic acid of the type described above. We shall give illustrations of suitable corrosion inhibiting compounds by reference to various patents and patent applications in which they are described, it being understood that the present application is based on the discovery of the enhancement of the corrosion inhibition exhibited by these compounds, rather than in the compounds themselves.

A particularly effective group of corrosion inhibiting agents are those described in Patent Re. 23,227, Blair and Gross. These compositions are cyclic amidines, particularly imidazolines characterized by having at least one hydrocarbon group containing 8 to 32 carbon atoms. The compositions may, and advantageously do, have in addition to the two nitrogen atoms which form part of the cyclic structure additional basic nitrogen atoms present as part of a side chain linked to one of the ring nitrogen atoms, as where the products are derived from triethylene tetramine, tetraethylene pentamine, or the high-boiling residues from the production of these compositions, having 6, 7 or even more amino groups. The compositions of this patent constitute one class of corrosion inhibitors which is usefully employed in preparing the compositions of the present application. Typical useful compounds of this type include:

2-undecylimidazoline;  
2-heptadecylimidazoline;  
2-pentadecyl, 1-heptylimidazoline;  
2-octyl, 1-hydroxyethylimidazoline;  
2-nonyl, 1-decylimidazoline;  
2-oleylimidazoline;  
2-cyclohexylethyl, 1-methylimidazoline;  
2-abietyl, 1-ethyloxyethylimidazoline;  
1-octadecylimidazoline;  
2-methyl, 1-octylimidazoline;  
1-dodecyloxymethyl, 2-hydroxymethylimidazoline;  
1-oleoyloxyethyl, 2-chloromethylimidazoline;  
1-N-decylaminoethyl, 2-ethylimidazoline;  
1-abietyl, 2-phenylimidazoline;  
2-heptadecyl, 1-aminoethylimidazoline;

2-heptadecyl, 1-diethylenediaminoimidazoline;  
2-methyl, 1-hexadecylaminoethylaminoethylimidazoline;  
1-dodecylaminopropylimidazoline;  
1-stearoyloxyethylaminoethylimidazoline;  
2-ethyl, 1-(N,N-dodecyl, hydroxyethyl)aminoethylimidazoline;  
1-stearamidoethylaminoethylimidazoline;  
1-(N-dodecyl)-acetamidoethylaminoethylimidazoline;  
Chloroparaffin alkylation product of 1-aminoethyl, 2-methylimidazoline.

Application Serial No. 227,944, filed May 23, 1951, Blair and Gross, now U.S. Patent No. 2,640,029, dated May 26, 1953, describes, as corrosion inhibitors, substituted tetrahydropyrimidines of the formula type:



where D is a member of the class consisting of D'-R and R; D' represents a divalent organic radical containing less than 25 carbon atoms, composed of elements from the group consisting of C, H, O, and N; R is a member of the class consisting of hydrogen and hydrocarbon radicals, with the proviso that at least one occurrence of R contains from 8 to 32 carbon atoms; B is a member of the class consisting of hydrogen and hydrocarbon radicals containing less than 7 carbon atoms, with the proviso that at least three occurrences of B be hydrogen. Typical substituted tetrahydropyrimidines of this type include:

2-undecyl, 4-methyltetrahydropyrimidine;  
1-ethyl, 2-octyl, 4-dimethyl, 6-cyclohexyltetrahydropyrimidine;  
2-heptadecyl, 6-methyltetrahydropyrimidine;  
2-abietyl, 4,6-dimethyltetrahydropyrimidine;  
2-naphthylmethyl, 1-butyltetrahydropyrimidine;  
2-cyclohexylethyl, 1,6-dimethyltetrahydropyrimidine;  
1-octadecyl, 2-methyltetrahydropyrimidine;  
1-oleylamidoethyltetrahydropyrimidine;  
1-stearoyloxyethyl, 4-phenyltetrahydropyrimidine;  
2-heptadecyl, 1-aminopropyltetrahydropyrimidine;  
Chloroparaffin alkylation product of 1-aminopropyl, 2-methyltetrahydropyrimidine;  
1-dipropylendiamino, 2-cyclopentylpropyltetrahydropyrimidine.

Application Serial No. 317,596, filed October 29, 1952, now abandoned, Blair, describes as corrosion inhibitors oxyethylated imidazolines such as compounds of the formula:



in which D represents a divalent, non-amino, organic radical containing less than 25 carbon atoms, composed of elements from the group consisting of C, H, O, and N; D' represents a divalent, organic radical containing less than 25 carbon atoms, composed of elements from the group consisting of C, H, O, and containing at least one amino group; and R is a member of the class consisting of hydrogen and aliphatic and cycloaliphatic hydrocarbon radicals; with the proviso that at least one occurrence of R contains 8 to 32 carbon atoms. Typical examples of such compounds having corrosion inhibiting properties include the products obtained by adding from

2 to 20 moles of ethylene oxide per mole to the following imidazolines, as described in said application:

2-undecylimidazoline;  
 2-heptadecylimidazoline;  
 2-oleylimidazoline;  
 2-heptadecyl, 4,5-dimethylimidazoline;  
 2-heptadecyltetrahydropyrimidine;  
 2-hydroxyethyl, 5-ethyl, 1-decytetrahydropyrimidine;  
 1-aminoethyl, 2-heptadecylimidazoline;  
 1-diethylenediamino, 2-heptadecylimidazoline;  
 1-triethylenetriamino, 2-ethylheptadecylimidazoline;  
 1-aminoethyl, 2-undecylimidazoline;  
 1-diethylenediamino, 2-undecylimidazoline;  
 1-triethylenetriamino, 2-undecylimidazoline;  
 1-aminoethyl, 2-pentadecylimidazoline;  
 1-diethylenediamino, 2-pentadecylimidazoline;  
 1-triethylenetriamino, 2-pentadecylimidazoline;  
 1-aminoethyl, 2-nonylimidazoline;  
 1-diethylenediamino, 2-nonylimidazoline;  
 1-triethylenetriamino, 2-nonylimidazoline;  
 1-aminoethyl, 2-heptadecenylimidazoline;  
 1-diethylenediamino, 2-heptadecenylimidazoline;  
 1-triethylenetriamino, 2-heptadecenylimidazoline;  
 1-aminoethyl, 2-undecenylimidazoline;  
 1-diethylenediamino, 2-undecenylimidazoline;  
 1-triethylenetriamino, 2-undecenylimidazoline;  
 1-aminoethyl, 2-hydroxyheptadecenylimidazoline;  
 1-diethylenediamino, 2-hydroxyheptadecenylimidazoline;  
 1-triethylenetriamino, 2-hydroxyheptadecenylimidazoline;  
 1-aminoethyl, 2-abietylimidazoline;  
 1-diethylenediamino, 2-abietylimidazoline;  
 1-triethylenetriamino, 2-abietylimidazoline;  
 1-aminoethyl, 2-cyclohexylethylimidazoline;  
 1-diethylenediamino, 2-cyclohexylethylimidazoline;  
 1-triethylenetriamino, 2-cyclohexylethylimidazoline;  
 1-aminoethyl, 2-naphthylimidazoline;  
 1-diethylenediamino, 2-naphthylimidazoline;  
 1-triethylenetriamino, 2-naphthylimidazoline;  
 1-aminopropyl, 2-heptadecyl(methyl\*)imidazoline; \*in 4 or 5 position  
 1-aminopropylaminopropyl, 2-haptadecyl(methyl\*)imidazoline; \*in 4 or 5 position  
 1-aminopropyl, 2-heptadecenyl(methyl\*)imidazoline; \*in 4 or 5 position  
 1-aminopropylaminopropyl, 2-heptadecenyl(methyl\*)imidazoline; \*in 4 or 5 position  
 1-aminopropyl, 2-undecenyl(methyl\*)imidazoline; \*in 4 or 5 position  
 1-aminopropylaminopropyl, 2-undecenyl(methyl\*)imidazoline; \*in 4 or 5 position  
 1-aminopropyl, 2-abietyl(methyl\*)imidazoline; \*in 4 or 5 position  
 1-aminopropylaminopropyl, 2-abietyl(methyl\*)imidazoline; \*in 4 or 5 position  
 1-aminopropyl, 2-naphthyl(methyl\*)imidazoline; \*in 4 or 5 position  
 1-aminopropylaminopropyl, 2-naphthyl(methyl\*)imidazoline; \*in 4 or 5 position

Application Serial No. 323,150, filed November 28, 1952, now abandoned, Blair, describes substituted carbonyl compounds containing at least two cyclic amidine radicals which are usefully used in preparing compositions of the invention, these being compounds in which the cyclic amidine radical is of the structure



wherein R is a hydrocarbon radical containing from 7 to 31 carbon atoms; n is the numeral 2 to 3 inclusive; R<sub>1</sub>

is a member of the class consisting of hydrogen atoms and lower alkyl radicals; R<sub>2</sub> is a member of the class consisting of alkylene radicals and lower alkyl substituted alkylene radicals; X is a member of the class consisting of amino radicals and amino alkylene-substituted amino radicals, with the proviso that there be at least one amino radical selected from the class of primary and secondary amino radicals; at least two such radicals in the final compositions, being united through amino nitrogens of the radicals X by at least one member of the class consisting of



15 and



20

radicals. Typical compositions of this type include compositions wherein

1-aminoethyl, 2-heptadecyltetrahydropyrimidine is coupled with urea;  
 25 1-aminopropyl, 2-heptadecyltetrahydropyrimidine is coupled with biuret;  
 1-dipropylenediamino, 2-heptadecyltetrahydropyrimidine is coupled with urea;  
 30 1-aminoethyl, 2-undecyltetrahydropyrimidine is coupled with guanidine carbonate;  
 1-aminopropyl, 2-undecyltetrahydropyrimidine is coupled with biuret;  
 1-dipropylenediamino, 2-undecyltetrahydropyrimidine is coupled with urea;  
 35 1-aminoethyl, 2-decyltetrahydropyrimidine is coupled with thiourea;  
 1-aminopropyl, 2-decyltetrahydropyrimidine is coupled with urea;  
 40 1-dipropylenediamino, 2-decyltetrahydropyrimidine is coupled with biuret;  
 1-aminoethyl, 2-heptadecylimidazoline is coupled with urea;  
 1-diethylenediamino, 2-heptadecylimidazoline is coupled with biuret;  
 45 1-triethylenetriamino, 2-pentadecylimidazoline is coupled with guanidine carbonate;  
 1-aminoethyl, 2-undecenylimidazoline is coupled with thiourea;  
 1-diethylenediamino, 2-undecenylimidazoline is coupled with urea;  
 50 1-triethylenetriamino, 2-undecenylimidazoline is coupled with biuret;  
 1-aminoethyl, 2-hydroxyheptadecenylimidazoline is coupled with thiourea;  
 55 1-aminoethyl, 2-cyclohexylethylimidazoline is coupled with urea;  
 1-triethylenetriamino, 2-abietylimidazoline is coupled with thiourea;  
 1-aminoethyl, 2-naphthylimidazoline is coupled with urea.

Patent 2,598,213, May 27, 1952, Blair, describes as corrosion inhibitors basic amides of polyamines characterized by the presence of an acyl radical of a carboxy acid having 8 to 32 carbon atoms and at least one basic amino nitrogen atom, that is, an amino radical characterized by freedom from directly linked aryl radicals and acyl radicals, which are useful as the corrosion inhibitor constituent of the new compositions.

70 Typical useful amino amides include the amide from 283 parts of stearic acid and 438 parts of triethylene tetramine; the amide from 381 parts of oleic acid with 584 parts of triethylene tetramine; the amide from 283 parts of stearic acid and 400 parts of the residue obtained by removing ethylene diamine from the heat and pres-

sure reaction of ethylene dichloride and ammonia; the amide from 300 parts of ricinoleic acid and the same mixture of bases; the amide from 100 parts by weight of olive oil and 100 parts by weight of diethylene triamine; the amide from 310 parts by weight of the ethyl ester of oleic acid and 286 parts by weight of triethylene tetramine; corresponding amides from purified naphthenic acids and from the carboxy acids derived by the oxidation of Pennsylvania crude oil; the amide from 284 parts of stearic acid and 74 parts of 1,2-propylene diamine.

Other effective inhibitors are the higher alkyl diamines such as N-octadecylpropylene diamine, and similar polyamines obtained by treating the monoamines corresponding to naturally occurring fatty acids or other mono-carboxy detergent-forming acids with acrylonitrile followed by hydrogenation to convert the nitrile group to an amino group. We have found the corrosion inhibiting properties of such compounds are enhanced when they are incorporated in compositions of the present invention.

From the foregoing it will be noted that there are a number of compounds characterized by the presence of at least two nitrogen atoms, at least one of which is basic, and a hydrocarbon group having 8 to 32 carbon atoms which have corrosion inhibiting properties, and which have their effectiveness substantially increased by association with an alkylated aromatic sulfonic acid of the type described above. The effectiveness of the corrosion inhibitors varies, some being considerably more effective than others, and so far as we are aware, there will be variation in effectiveness of the compositions of the invention more or less parallel to the variations in effectiveness of the corrosion inhibitors per se. We believe that the most effective of the corrosion inhibitors are the complex cyclic amidines, in particular the substituted glyoxalidines described in Patent Re. 23,227, and the complex amidines described in applications Serial Nos. 227,944, 317,596 and 323,150, together with the amino amide products described in Patent 2,598,213.

We have heretofore referred to the fact that the new compositions of the invention may be used in liquid form, usually with the use of an appropriate solvent such as a mixture of high boiling aromatic hydrocarbons and medium boiling paraffinic hydrocarbons or may be used in stick form with or without weighting agents. The use of corrosion inhibitors in stick form and in weighted stick form, the purpose of providing them in such form, and the preparation of products in such form is well known. See, for example, Patents 2,599,384 and 2,599,385, June 3, 1952. The compositions of the present invention may be used as the corrosion inhibiting constituents of weighted solid stick inhibitors as described in these patents or of non-weighted solid stick inhibitors.

The invention will be further illustrated by the following specific examples in which typical compositions of the invention are described. In each of them, we have found that the corrosion inhibiting action of the corrosion inhibitor is markedly enhanced by the alkylated aromatic sulfonic acid associated with it. This enhancement is also found with the wide range of inhibitors described above and the examples are, therefore, given purely by way of illustration and not by way of limitation.

#### Example I

320 lbs. of refined tall oil and 146 lbs. of triethylene tetramine were heated and stirred in an autoclave for 2½ hrs. after reaching a temperature of 285° C. Approximately 36 lbs. of water were evolved during the reaction. The product consisted largely of 1-aminoethylaminoethylimidazoline substituted in the 2-position by hydrocarbon residues originally attached to the —COOH groups of the fatty acids and rosin acids of the tall oil. To 100 lbs. of the above product were added 190 lbs. of high boiling aromatic gas oil. While stirring this solution, 12 lbs. of anhydrous glycolic acid were added slowly. Finally, 100 lbs. of a 50% (by wt.) solution of am-

monium diisopropyl naphthalene sulfonate in an 80-20 mixture of aromatic gas oil and isopropyl alcohol were added while stirring. The finished compound was a thin oil.

5

#### Example II

384 lbs. of tall oil and 146 lbs. of triethylene tetramine were reacted for 2½ hrs. at 285° C., as described in Example I. Approximately 41.5 lbs. of water were evolved and condensed from the autoclave. The product 10 consisted of a mixture of mono- and di-imidazolines with minor proportions of substituted amides of tall oil fatty acids. To 100 lbs. of this product were added 191 lbs. of aromatic gas oil and, while stirring, 9 lbs. of 66° Baumé sulfuric acid at such a rate as to maintain a 15 temperature of less than 100° C. and above 80° C. Some heat may be applied if necessary to maintain this temperature. 100 lbs. of a 50% (by wt.) solution of ammonium diisopropyl naphthalene sulfonate in an 80-20 mixture of commercial xylene and isopropyl 20 alcohol were added to the above and the whole stirred until homogeneous.

#### Example III

50 lbs. of ammonium diisobutyl naphthalene sulfonate 25 were substituted for the ammonium diisopropyl naphthalene sulfonate of Example II.

#### Example IV

50 lbs. of the cyclohexylamine salt of diisobutyl naphthalene sulfonic acid were substituted for the ammonium diisopropyl naphthalene sulfonate of Example II.

#### Example V

The polyethylene polyamine reactant used in the 35 preparation of the corrosion inhibitor portion of this product consisted of the high-boiling still residue remaining after distillation of lower boiling polyamines, up to and including tetraethylene pentamine, resulting from the condensation of ethylene dichloride and ammonia. This residual polyamine contained 33.5% nitrogen and 40 consisted of a mixture of pentaethylenehexamine and higher homologs. 52 lbs. of the above described polyamine and 100 lbs. of commercial California naphthenic acid of acid number 234 were reacted at 280° C. for 4 hours. To this corrosion inhibitor product were added, 45 with stirring, 150 lbs. of kerosene, 20 lbs. of linoleic acid, and 50 lbs. of cyclohexylammonium dodecyl benzene sulfonate.

#### Example VI

50 A solid stick type corrosion inhibitor with improved 55 activity was prepared by casting the homogeneous melt resulting from mixing the following ingredients at 100-120° C.:

Corrosion inhibitor of Example V \_\_\_\_\_ lbs. 50  
55 Ammonium diisopropyl naphthalene sulfonate \_\_\_\_\_ lbs. 10  
Microcrystalline wax of 186° F. M.P. \_\_\_\_\_ lbs. 40  
Oxidized microcrystalline wax of 185° F. M.P. and  
60 saponification value \_\_\_\_\_ lbs. 20

The solid product has a density of about 0.93 at 25° C.

#### Example VII

A solid stick type corrosion inhibitor of high density 65 particularly useful in the treatment of distillate wells prepared by casting the melt resulting from mixing thoroughly the following ingredients at about 120° C.:

Product of Example VI \_\_\_\_\_ lbs. 38  
70 Powdered barium sulfate \_\_\_\_\_ lbs. 62

The solid product had a density of about 2.0 and a 75 softening point of about 180° F.

#### Example VIII

The sulfonic acid component of this composition was prepared as follows:

600 lbs. of a naphthenic type crude oil of 22 API

gravity were run into a lead lined sulfonating tank, equipped with stirrer, heater coils and drain lines. While stirring and maintaining the oil at 35° C., 300 lbs. of 20% oleum were run into the oil over a period of 3 hrs. The mixture was then stirred for an additional 30 minutes, heated to 90° C. and washed by adding 20 gals. of water. After settling quietly for 4 hrs., the acidic water layer was drawn off and the oil layer neutralized to the methyl orange end point by addition, with stirring, of aqua ammonia (approximately 29% NH<sub>3</sub>).

100 lbs. of this component were mixed with 800 lbs. of the tall oil reaction product of Example II. This mixture was warmed to 80° C. and stirred until homogeneous.

The following is a typical illustration of the enhancement of the corrosion inhibiting action obtained with the compositions of the present invention:

Weighed plates of 1020 steel were rotated in a mixture of 55 ml. of kerosene, and 250 ml. of a brine containing 2% sodium chloride, 0.2% sodium sulfate, 0.4% calcium chloride and 0.4% magnesium chloride hexahydrate. The stirring apparatus was maintained at a temperature of 100° F. in a controlled atmosphere of 0.25 atmosphere of hydrogen sulfide and 0.75 atmosphere of nitrogen. The plates were rotated for a period of 72 hours, after which they were removed, dipped briefly in inhibited HCl to remove ferrous sulfide, washed, dried and weighed to determine loss of metal. Parallel tests were run using no inhibitor, using 160 parts per million of the tall oil reaction product of Example II, using 160 parts per million of the same inhibitor with 16 parts per million of ammonium diisopropyl naphthalene sulfonate, using 160 parts per million of the same inhibitor and 40 parts per million of the same sulfonate, using 160 parts per million of the same inhibitor and 80 parts per million of the same sulfonate, and using no inhibitor but 160 parts per million of the same sulfonate. The average weight loss from tests run in quadruplicate showed 241 mg. with no added agent, 185 mg. with the sulfonate only, 43 mg. with the inhibitor only, 16 mg. with the inhibitor plus 16 parts per million of sulfonate, 20 mg. with the inhibitor plus 40 parts per million of the sulfonate and 14 mg. with the inhibitor plus 80 parts per million of the sulfonate. Similar results were obtained in other laboratory tests using various brine-oil combinations, various corrosive atmospheres, and various combinations of inhibitor and sulfonate.

In another test, carried out under the same conditions, but with a 48 hour test period, the weight loss of the 1020 steel plates was 166 mg. with no added agent, 164 mg. with 40 parts per million of ammonium diisopropyl naphthalene sulfonate, 35 mg. with 40 parts per million of N-aminopropyl octadecylamine, 17 mg. with 40 parts per million of this same amine and 7 parts per million of the sulfonate, 17 mg. with 40 parts per million of the amine and 30 parts per million of the sulfonate and 16 mg. with 40 parts per million of the amine and 40 parts per million of the sulfonate.

The effectiveness of the compositions in the field was shown by the results of a test in a gas distillate well in the Gwinville field in Mississippi. This well produced three million cubic feet of gas, 40 barrels of liquid hydrocarbon and five barrels of salt water a day. Before treatment, water trapped from the flow line at the surface showed an iron content of about 240 parts per million.  $2\frac{1}{2}$  gallons of the tall oil reaction product of Example II, dissolved in  $7\frac{1}{2}$  gallons of hydrocarbon condensate were introduced down the annulus between the casing and the tubing once each week. It flowed down the annulus, became mixed with the produced fluids at the bottom of the hole and was carried up the tubing to the surface by the gas flow. After several weeks of such treatment, the water from the flow line had an iron content of 50-60 parts per million.  $2\frac{1}{2}$  gallons of the prod-

uct of Example II were then substituted for this inhibitor, and used in the same way. After three weeks, the water was found to have an iron content of 10-15 parts per million.

5 In the foregoing we have referred at length to the inhibitors which are used as being compounds having at least two nitrogen atoms, at least one of which is basic, and at least one hydrocarbon group having 8 to 32 carbon atoms. It is to be understood that these compositions  
10 may be used in the form of the free bases, or in partially neutralized form or in completely neutralized form, and such partial or complete neutralization may be by means of an inorganic acid, such as sulfuric acid, or an organic acid, such as acetic acid, gluconic acid, a  
15 higher fatty acid or any of the acids which are used for neutralizing basic amino corrosion inhibitors, in accordance with usual practice.

An additional advantage in the use of the new compositions which we have observed is a substantial and unexpected decrease in certain emulsification problems sometimes encountered. Thus, when corrosion inhibitors of the type used in the compositions of the invention are incorporated in hydrocarbon-water systems where the hydrocarbon is relatively pure, i.e., is gasoline, kerosene, distillate, liquefied petroleum gases and the like, as contrasted with crude oil, there is a tendency for oil-in-water emulsions to form. This tendency is greatly reduced, or absent, when the new compositions are used. This is surprising, because the alkylated aromatic sulfonates, while known to resolve water-in-oil emulsions, have found no application as demulsifiers for oil-in-water emulsions.

We claim:

The process of inhibiting corrosion of ferrous metals exposed to corrosive agents normally present in producing oil and gas wells which includes introducing into the well a composition having corrosion inhibiting properties which contains, as an active corrosion inhibiting constituent, a nitrogen-containing agent characterized by having at least 2 nitrogen atoms, at least one of which is basic, and at least one hydrocarbon group having 8 to 32 carbon atoms and which contains, in admixture therewith, as an agent which enhances the corrosion inhibiting activity of the corrosion inhibiting constituent, at least 5% and not over 100% based on the corrosion inhibiting constituent, of an alkylated aromatic sulfonic acid compound selected from the class consisting of alkylated naphthalene sulfonic acid compounds of the formula



55 in which R is an alkyl radical having 3 to 12 carbon atoms, n is a number from 1 to 3, with the proviso that the total number of carbon atoms present in  $(R)_n$  is at least 6, and alkylated benzene sulfonic acid compounds of the formula



in which  $n$  is a number from 1 to 2, R is an alkyl group having 3 to 18 carbon atoms, with the proviso that the total number of carbon atoms in  $(R)_n$  is at least 9.

**References Cited in the file of this patent**

UNITED STATES PATENTS

|    |           |                      |               |
|----|-----------|----------------------|---------------|
| 70 | 2,493,483 | Francis et al. ----- | Jan. 3, 1950  |
|    | 2,583,399 | Wachter -----        | Jan. 22, 1952 |
|    | 2,618,608 | Schaeffer -----      | Nov. 18, 1952 |
|    | 2,658,036 | Core et al. -----    | Nov. 3, 1953  |